

J. M. HYDE.  
PROCESS OF SMELTING ZINC ORES.  
APPLICATION FILED FEB. 13, 1914.

1,118,012.

Patented Nov. 24, 1914.

2 SHEETS—SHEET 1.

Fig. 1.



Fig. 2.



Inventor

Witnesses

E. Daniels

P. J. Fulsiger.

James M. Hyde

By Beynes, Townsend & Brickhouse  
Attorneys

1,118,012.

J. M. HYDE.  
PROCESS OF SMELTING ZINC ORES.  
APPLICATION FILED FEB. 13, 1914.

Patented Nov. 24, 1914.

2 SHEETS—SHEET 2.

Fig. 3.



Fig. 4.



Witnesses

E. Daniels  
R. J. Hulsaizer.

By

James M. Hyde  
Byrnes, Townsend & Brickerstein  
Attorneys

# UNITED STATES PATENT OFFICE.

JAMES M. HYDE, OF BERKELEY, CALIFORNIA.

## PROCESS OF SMELTING ZINC ORES.

1,118,012.

Specification of Letters Patent. Patented Nov. 24, 1914.

Application filed February 13, 1914. Serial No. 818,576.

To all whom it may concern:

Be it known that I, JAMES M. HYDE, a citizen of the United States, residing at Berkeley, in the county of Alameda and State of California, have invented certain new and useful Improvements in Processes of Smelting Zinc Ores, of which the following is a specification.

My invention relates to a method of smelting metal-bearing materials containing zinc or any other volatilizable metal or metallic compound, and especially that class of ores containing zinc and other metals such as lead, copper, gold, and silver; and has for its object to recover such other metals in a molten state while at the same time the zinc or other volatilizable metal or metallic compound is vaporized, and recovered. This object I attain by smelting the charge over a bath of slag or matte and out of contact with the gases of combustion used for producing the smelting heat.

The smelting operation may be carried out in furnaces such as are shown in the accompanying drawings, in which—

Figure 1 is a vertical, transverse section through one type of furnace; Fig. 2 is a partial longitudinal section; Fig. 3 is a transverse section through a modified form of furnace; and Fig. 4 is a vertical longitudinal section.

Referring to Fig. 1, A is the furnace wall inclosing the heating-chamber and the retort structure B, which may be made of any material resistant to heat and the corrosive action of slag or matte, such as clay, silica, magnesite or basic bricks, chromite or carborundum, or of bricks or blocks coated with chromite, carborundum or other suitable material. In its lower portion, the structure B is provided with open arches C which permit the fused material to pass out into and fill the lower portion of the furnace A, which is provided with tap-holes D, E, F, for slag, matte, and base bullion, respectively. The level of the matte or slag bath is maintained above the tops of the arches, so that the products of combustion from the gas burners G and H or other heating means have no access to the charge within the retort B. I is a flue leading to a stack for carrying off the waste gases. The retort B has an upper portion K extending above the furnace and provided with a charging-hopper L. M, M are pipes for leading off the zinc vapors and N, N are condensers there-

for. 10 is an internal, longitudinally arranged arch providing a heating-chamber beneath the charge and above the slag, and provided with a burner G'' for furnishing 60 additional heat to the charge through the arch and directly to the slag. This arch performs the further function of acting as a support for the charge.

In the modified form of furnace shown in Fig. 2, a perforated or open-bottomed retort B' extends transversely across the furnace chamber. The ore is delivered through the hopper P' into a charging-tube L' in which is mounted a screw-conveyer O' for forcing 70 the material into the retort B' which, at its opposite end, is provided with a tube M' for conveying zinc vapors to the condenser N'. Instead of a single retort B', a series of retorts may be used, which are supported upon 75 a suitable structure R', provided, as in Fig. 1, with open arches C', which permit the molten mass to flow into the lower portion of the furnace proper A', which is provided with slag, matte, and base bullion taps D', 80 E', F'.

The operation of the process as carried out in the form of furnace shown in Fig. 1, is as follows:—The charge of ore, mixed with the proper fluxes and reducing-agents, either 85 loose or briqueted, is fed through the hopper L into the stack portion K of the retort B. As it passes downwardly, it is heated by the flame outside the retort and by heat from the arch 10, and is finally reduced and 90 fused, the fused mass filling the lower portion of the retort and furnace to a point above the tops of the arches C, this fused mass thus acting as a liquid seal and preventing direct access of the products of combustion to the ore charge. The descending column of ore is of such height and density that the volatilized zinc which has a free 95 exhaust from the smelting chamber into the condenser or conduit to the oxidizing 100 chamber and bag house, will follow that course and will not pass out upward through the descending charge and be lost, nor will atmospheric oxygen enter the smelting zone 105 through the descending charge. As a result of this smelting operation, the zinc is reduced and volatilized and the other metallic 110 contents of the charge are collected in the molten bath formed in the lower portion of the furnace. The lead will be reduced and, with some of the gold and silver, will form a layer of base bullion at the bottom. The

copper will form a layer of matte also containing some gold or silver, superincumbent on the lead; and resting on the layer of matte, will be a layer of slag. If necessary, 5 granulated matte, sulfids, or cement copper may be added to the charge to assist in the formation of a matte. Cement copper would also act as a reducing agent, breaking up any zinc sulfid left in the charge.

10 The volatilized zinc is delivered through the pipes M to the condensers N, in which it is condensed to molten spelter, and from which it may be removed in any suitable manner. Where metallic zinc is desired, the 15 zinc-bearing ore, if a sulfid, should be roasted, or if a carbonate, should be calcined, so that, as far as possible, the zinc shall exist in the charge as an oxid. When zinc oxid is to be produced, air may be admitted to 20 the vapors driven off from the charge and the thus-produced zinc oxid carried to a bag house or otherwise collected, as by an electrostatic fume arrester. If desired or necessary, reducing-gases may be introduced 25 into the zinc vapors as they pass to the zinc condensers. The process is carried out in the furnace shown in Fig. 2, in substantially the same way.

It will be noted that in my process the 30 charge is not directly subjected to combustion gases and the oxidation of the zinc, and the volatilization and oxidation of the lead, are thereby prevented, the lead and zinc being separately collected, the zinc in 35 the form of spelter or oxid and the lead as base bullion. It will be noted further that heat is supplied to the charge to be melted indirectly through the walls of the retort while the surface of the molten material 40 outside the retort is directly subjected to the action of the heat and flame in the combustion chamber. This molten material is therefore directly heated and serves to convey heat directly to that portion of the 45 charge in contact with such molten material within the retort. The slag, matte, and base bullion may be tapped off directly, either continuously or intermittently, or instead of being separately tapped from the 50 furnace, the whole fused mass may be passed into a fore-hearth and slag, matte, and bullion there separated in the well-known way.

In the process of the recovery of zinc 55 from its ores by the use of the retort furnace which is now the standard method of zinc-recovery, the consumption of labor, fuel, and refractory materials is high, the capacity of the furnace is low, because the units used are necessarily small, and the 60 furnace work is intermittent or cyclic, and it is necessary to treat, in an independent operation, the residues left after the zinc is recovered, which are in many cases of value because of their content of lead, copper, and the precious metals. A further

disadvantage exists in that certain types of ores and concentrates contain mineral materials which flux and destroy the clay retorts in which the ore is treated.

My process herein disclosed produces 70 great economy in all of the essential features of zinc-treatment. The amount of fuel which is required is less than that now consumed in regular practice, as the process is in most cases continuous for a considerable period of time and there are not therefore those heat losses which are occasioned by shutting down and discharging and charging an ordinary retort furnace. Further, the waste heat from the smelting- 75 operation is used for the heating of the advancing charge approaching the smelting zone and may be still further used after leaving the furnace for the production of steam for power use. As the furnace is not 80 intermittently heated and cooled, the expansion and contraction of the retorts which takes place in the ordinary zinc furnace, is avoided, and results in considerable economy of materials, as the life of the retorts 85 is greater. The material of the charge which ordinarily forms a residue requiring further and independent treatment if it contains valuable metallic constituents, is, 90 by my process, smelted in a single operation and from it may be recovered its content of copper, lead, and the precious metals in concentrated and commercially desirable form, as in mattes, and base bullions.

It is to be understood that by the term 100 "zinc," as used in the specification and claims, is included any other material or materials susceptible of treatment by the described process; and that by the term "ore," as used in the claims, is meant not 105 only ore, but any metal-bearing material, such as slag, concentrates, etc. The slags or matte forming the molten bath in the furnace may be either that produced by the smelting operation, or if such slag or matte 110 is of insufficient amount, may be augmented by additions of already formed slags or mattes, either in solid or molten condition.

I do not herein claim the novel furnace hereinbefore described but reserve the right 115 to file a subsequent application therefor.

I claim:

1. The process of smelting zinciferous ores, which consists in heating the ore mixed with flux and reducing-agent in an externally 120 heated retort to a temperature sufficient to reduce the metallic constituents, collecting the molten materials in a bath beneath the charge, removing the zinc vapors from the retort above the molten bath, and keeping 125 the bath molten by heat directly applied to the surface thereof outside said retort.

2. The process of smelting zinciferous ores, which consists in heating the ore mixed with flux and reducing-agent in an externally 130

- heated retort to a temperature sufficient to reduce the metallic constituents, collecting the molten materials in a bath beneath the charge, removing the zinc vapors from the 5 retort above the molten bath, keeping the bath molten by heat directly applied to the surface thereof outside said retort, and separately removing the base bullion, matte and slag.
- 10 3. The process of smelting zinciferous materials by heating such materials out of contact with products of combustion to a reducing temperature over a bath of matte or slag kept molten by heat directly applied 15 to a portion thereof, and removing the zinc vapors from above the molten bath.
4. The process of smelting zinciferous ores which consists in heating the ore mixed with flux and reducing agent in an externally 20 heated retort to a temperature sufficient to reduce the metallic constituents, collecting the molten materials in a bath beneath the charge, removing the zinc vapors from the retort above the molten bath, condensing 25 the zinc vapors to spelter, and keeping the bath molten by heat directly applied to a portion of the surface thereof outside of said retort.
5. The continuous process of smelting 30 zinciferous ores which consists in continuously feeding the ore mixed with proper flux and reducing agent into an externally heated retort and smelting the mixture therein out of contact with the products of 35 the combustion of the fuel whereby it is heated, removing the volatilized zinc, and removing from the smelting chamber during the smelting operation the remaining constituents of the charge in molten condition.
- 40 6. The continuous process of smelting zinciferous ores which consists in continuously feeding the ore mixed with proper
- flux and reducing agent into an externally heated retort, smelting the mixture therein 45 out of contact with the products of the combustion of the fuel whereby it is heated, continuously removing and condensing the volatilized zinc, and removing from the smelting retort during the smelting operation 50 the remaining constituents of the charge in molten condition.
7. The process of smelting zinciferous ores which consists in continuously feeding the ore mixed with proper flux and reducing 55 agent into an externally heated retort, smelting the mixture therein out of contact with the products of combustion of the fuel whereby it is heated, continuously removing the volatilized zinc, as a vapor, removing 60 the other constituents of the charge in a molten condition during the smelting operation and keeping said molten products of the smelting operation in the form of a molten bath by heat directly applied to the surface 65 of the molten bath outside of the retort in which smelting takes place.
8. The continuous process of smelting zinciferous ores, which consists in feeding ore mixed with the proper flux and reducing agent into an externally heated retort and smelting the mixture therein out of contact with the products of combustion of the fuel whereby it is heated, and maintaining 70 an adequate supply of ore and flux during 75 the smelting, removing the volatilized zinc and removing from the smelting chamber during the smelting operation the remaining constituents of the charge in a molten condition.
- 80 In testimony whereof I affix my signature in presence of two witnesses.

JAMES M. HYDE.

Witnesses:

Jos. H. BLACKWOOD,  
J. H. BRICKENSTEIN.